

Feb. 11, 1930.

G. F. MURPHY

1,747,125

ROAD AND STREET CONSTRUCTION

Filed June 6, 1928

*Fig. 1.*



*Fig. 2.*



*Fig. 3.*



INVENTOR  
*G.F. Murphy,*  
BY  
*Murphy & Co.*  
ATTORNEY

## UNITED STATES PATENT OFFICE

GUY F. MURPHY, OF CORAL GABLES, FLORIDA

## ROAD AND STREET CONSTRUCTION

Application filed June 6, 1928. Serial No. 283,419.

This invention relates to a road construction.

An object of the invention is the provision of a road and street construction, and a process of forming the same, in which bituminous rock is crushed so that it will pass through a sieve of predetermined mesh and then rolled cold on a proper foundation of a road bed to form a base or levelling course, after which the ground bituminous rock is applied as a wearing surface.

A further object of the invention is the provision of a road and street construction and method of forming the same in which crushed bituminous rock, or a mixture of bituminous rock and clean hard stone, granite, or slag is mixed with the bituminous rock to form a levelling course after which the wearing surface is formed of ground bituminous rock rolled cold upon the levelling surface.

This invention will be best understood from a consideration of the following detailed description in connection with the accompanying drawings; nevertheless, it is to be understood that the invention is not confined to the disclosure being susceptible of such changes and modifications as shall define no material departure from the salient features of the invention as expressed in the appended claim.

In the drawings:—

Figure 1 is a transverse vertical section of a road constructed according to the principles of my invention.

Figure 2 is a fragmentary vertical section of a modified form of a road shown in Fig. 1.

Figure 3 is a fragmentary transverse section of a road showing a further modified form of the invention.

Referring more particularly to the drawings 10 and 11 designate a pair of concrete shoulders running longitudinally and located at the side edges of the road. Intermediate 45 these shoulders is formed a base 12 which may consist of crushed rock, concrete or any suitable material of predetermined depth and rolled to form a compact foundation.

Located upon the top of the base or foundation 12 is a layer 13 formed of crush bitu-

minous rock of a predetermined depth which is suitable for the needs which is known as a levelling surface. A wearing surface is shown at 14, and is formed of ground bituminous rock and rolled while cold.

55

Referring more particularly to Fig. 2, a base 20 is formed of any suitable material and is rolled to provide a compact foundation. Upon this base is rolled, while cold, a levelling surface 21, which is formed of equal parts of ground bituminous rock and clean, hard stone, granite or slag. The material forming the levelling surface must pass through a one inch mesh sieve, or screen.

60

Rolled upon the levelling surface 21 is a surface 22 known as the wearing surface and formed of ground bituminous rock.

65

Referring more particularly to Fig. 3, it will be found that the base and the levelling surface have been combined into a unitary structure, as indicated at 30, and formed of bituminous rock, which has been crushed to pass through a two and one-half inch mesh screen. A wearing surface 31 is applied to the top of the base 30 and consists of ground rolled bituminous rock which is ground in order to provide for a fine texture of material.

70

All materials are applied by the cold process and are laid just as the materials come from the producer, no artificial heat being applied for the purpose.

75

The levelling course indicated at 13 in Fig. 1 consists of crushed bituminous rock which has been passed through a one inch mesh screen and must be free of any foreign matter. 85 The asphalt content of the bituminous rock of this course should average not less than three (3) per cent or more than six and one-half (6½) per cent loss by ignition when determined by the official ignition method. The thickness of this course when compressed should not be less than approximately one inch nor more than one and one-half inches. However, the thickness of the course depends upon the type of traffic which the road is 90 designed to serve. The bituminous rock may be spread or levelled off manually or with a blade, or by means of the usual grader. When the crushed bituminous rock is raked off by hand, it is dumped in piles and shovelled into 95 100

place. Each succeeding shovel full is deposited next to the preceding pile, while maintaining the surface considerably higher than the required thickness of the loose material in order to permit the workman to rake the materials and maintain the proper grade. The raking continues until the entire surface has a uniform thickness throughout. When a blade or grader is employed for spreading the levelling course, the materials are deposited in piles and then shovelled into position after which the grader is run over the surface until a uniform thickness is had throughout the surface. During the raking of the materials, it is necessary that the workman keep off the raked surface in order to prevent a non-uniformity of the coating.

After a sufficient amount of surface of the proper thickness of the loose materials has been raked to allow for rolling, a self-propelled roller, which may be a tandem, or the three wheel type, weighing approximately five to eight tons is operated over the surface. In any event, the roller must be equipped with snugly fitting ash pans and provided with scrapers for maintaining the wheels clean.

In order to attain the uniformity of thickness of the levelling surface, it is necessary to operate the roller along lines which are parallel to the center-line of the road bed, beginning with the outer edge of the road bed and gradually working towards the center of the road, each succeeding strip of rolled material being overlapped with the preceding rolled strip of levelling surface for approximately one-third the width. This rolling operation in the manner just described, should be continued until the surface has been thoroughly bonded and compacted.

Where certain portions of the road bed show uneven surfaces, the roller may again be applied, but moved at an angle of forty-five degrees or diagonally across the street from each side. The surface is now ready for the application of the wearing surface. The materials from which the wearing surface is formed consists of finely ground bituminous rock which should meet the following requirements. First: The materials must be free of all foreign matter. Second: The asphalt content of the rock should be such that when tested according to the official ignition method, the representative sample should lose not less than six and one-half per cent. Third: The materials should be capable of passing through a screen one inch 90%, three-quarter inch 80%, one-half inch 70%. The thickness of the wearing surface should be not less than one-half inch and not more than one and one-half inches, the thickness, of course, depending upon the type of traffic it will have to serve.

This ground bituminous rock is located in piles and shovelled into place in such a man-

ner that each succeeding shovel full should be deposited in close association with the preceding, while the thickness of the materials in the loose state should be considerably higher than the required thickness of the loose materials, in order to enable the materials to be raked to the proper grade. The raking operation follows immediately the shovelling of the materials onto the levelling surface. Care is taken that the materials are uniformly distributed over the road bed. After the materials have been raked in position, care must be taken that no traffic is permitted of any kind on the loose materials.

If the materials forming the wearing surface are dry, and the atmospheric temperature is approximately fifty degrees F., or above rolling may be proceeded with immediately as fast as sufficient amount of materials are evenly applied to the levelling surface to enable the roller to operate. Where the temperature is below fifty degrees F. and the atmosphere appears damp, the surface should be permitted to dry and heated by the sun's rays before the rolling operation in order to provide for a perfect bond with the levelling course. This rolling operation is proceeded with on the same lines as has been described for the rolling of the levelling course.

Roller marks should be obliterated, and any honeycomb spots appearing after the first rolling operation must be filled in with sifted material which may pass through a one quarter inch sieve. Where a delay occurs between the application of the wearing surface on the levelling surface, the surface of the levelling course must be cleaned so that it will be free of dust or any foreign material, and furthermore, the surface of the levelling course should be free of moisture.

Where an old base or surface that is substantial is used, and is smooth, an asphalt primer or paint should be applied before the levelling course has been laid. This improved method of bituminous rock construction may be used for heavy traffic on streets or highways and may be employed to surface brick, concrete, asphalt or wooden block surfaces. In the application of the materials shown in Fig. 2, a slightly different procedure is required, due to the difference in the nature of the materials employed. The levelling course in this construction is composed of equal parts of bituminous rock used in the wearing surface, and any hard aggregate such as slag, lime stone, or granite. In this case the hard aggregate must be free of foreign matter and dust and of a size to pass a one inch mesh sieve. Equal parts of the slag, lime stone, or granite and bituminous rock, should be mixed together in any appropriate manner such as by hand, or by means of a revolving or concrete mixer. After the ground bituminous rock, and the mineral aggregate have been thoroughly mixed, they are applied to the base

of the road bed in the same manner as has been explained in reference to the application of the bituminous rock for forming the levelling course. The top coat or wearing surface is formed of ground bituminous rock applied in the manner described for the application of the wearing surface of the road bed shown in Fig. 1.

The road bed shown in Fig. 3 has a base formed of crushed bituminous rock and a wearing surface of ground bituminous rock thus eliminating the foundation or base indicated respectively at 12 and 20 in Figs. 1 and 2. However, the base member indicated at 30 in Fig. 3, consists of large particles of the crushed bituminous rock and they are of such size that the particles will pass through a two and one-half inch mesh screen. The test for the asphalt content should not average less than three nor more than six and one-half per cent loss by ignition when determined by the official ignition method by means of a representative sample of rock asphalt.

In this case, as in all other cases, the bituminous rock should be free of all foreign materials and moisture. After the subgrade is prepared, this rock shall be placed and spread to a depth of not over four inches in a loose state at one spreading. A ten ton, three wheel roller is employed for compacting the rock and the rolling operation should start along the edges and working towards the center. Two complete rollings over the surface should be sufficient for the purpose. After the rolling operation has been completed a second layer is spread over the first compact layer and thoroughly rolled. The top wearing surface formed of ground bituminous rock is then applied in the manner previously described.

I claim:—

A road construction comprising a base formed of a cold rolled layer of crushed rock, a cold rolled layer or levelling course on the crushed rock and formed of crushed bituminous rock which will pass through a one inch mesh screen and having an asphalt content of not less than three per cent or not more than six and one-half per cent loss by ignition when determined by the official ignition method, and a top layer of cold rolled ground bituminous rock in which seventy per cent will pass through a one-half inch mesh screen.

GUY F. MURPHY.